

## UNITED STATES PATENT OFFICE

JOHN A. GANN, OF MIDLAND, MICHIGAN, ASSIGNOR TO THE DOW CHEMICAL COMPANY, OF MIDLAND, MICHIGAN, A CORPORATION OF MICHIGAN

## MAGNESIUM BASE ALLOY

No Drawing.

Application filed April 25, 1932. Serial No. 607,509.

The present invention relates to improved light weight alloys in which magnesium is the predominating constituent. One object of my invention is to produce magnesium base alloys possessing the characteristic low specific gravity approaching that of magnesium that at the same time possess a combination of useful properties such as to make these alloys valuable for use in the mechanical arts. 10 Other objects and advantages will appear as the description proceeds.

Heretofore most of the commercial magnesium base alloys that possess high tensile strength contained aluminum as an essential 15 alloying ingredient. Although aluminum in combination with certain other alloying elements imparts valuable mechanical properties to magnesium base alloys, it has the disadvantage of decreasing the corrosion resistance when present in adequate amounts to impart high tensile strength. Moreover, this element very materially reduces the quantity of other elements, particularly manganese, which may be alloyed with magnesium at the 20 same time. Thus the valuable properties which manganese imparts to magnesium alloys cannot be fully realized when aluminum is present as a principal alloying ingredient.

Many attempts have been made to produce 25 high strength magnesium base alloys which do not contain aluminum and which at the same time are resistant to corrosion. Malleable alloys of this type are described in a copending application, Serial No. 593,193, filed February 15, 1932, which consist of a 35 ternary combination of magnesium with cadmium and zinc as alloying ingredients. I have now discovered that manganese can be alloyed more readily with the aforesaid magnesium-cadmium-zinc alloys than with those 40 alloys containing aluminum, and useful alloys are thereby produced which are not only superior to the parent ternary and binary alloys, but also possess a tensile strength which is substantially as high as any previously 45 known commercial magnesium base alloy, as well as a high degree of corrosion resistance.

Accordingly the alloys which are the subject of my invention contain the metals magnesium, cadmium, zinc, and manganese,

wherein the magnesium content exceeds 75 per cent, the cadmium, zinc, and manganese are each present in amounts of over 0.1 per cent and the quantity of the three metals cadmium, zinc, and manganese together is less than 25 per cent of the total. 55

Examples of my new improved quaternary alloys are given in the table showing their properties measured on extruded samples of the alloys, together with the properties of the 60 parent binary alloys of magnesium and manganese, and those of the parent ternary alloys of magnesium, cadmium, and zinc for comparison.

Table

65

| Alloy composition                           | Mechanical properties           |                            |                     |
|---------------------------------------------|---------------------------------|----------------------------|---------------------|
|                                             | Tensile strength<br>lbs./sq.in. | Yield point<br>lbs./sq.in. | Hardness<br>Brinell |
| 1. Binary alloy: Mg 99%, Mn 1%.             | 36,600                          | 21,800                     | 39                  |
| 2. Ternary alloy: Cd 2%, Zn 2%, balance Mg. | 32,000                          | 19,200                     | 41                  |
| 3. Quaternary alloy: Ditto (2), plus 1% Mn. | 41,200                          | 32,400                     | 56                  |
| 4. Ternary alloy: Cd 6%, Zn 2%, balance Mg. | 37,500                          | 22,500                     | 44                  |
| 5. Quaternary alloy: Ditto (4), plus 1% Mn. | 39,400                          | 27,600                     | 47                  |
| 6. Ternary alloy: Cd 4%, Zn 4%, balance Mg. | 37,300                          | 22,200                     | 41                  |
| 7. Quaternary alloy: Ditto (6), plus 1% Mn. | 41,300                          | 29,500                     | 52                  |

70

80

The data of the table indicates that the tensile strength, yield point (defined as the load in lbs./sq. in. at which the stress-strain curve deviates 0.1 per cent elongation from the modulus line) and hardness are improved in my new alloys compared to the previously known simpler parent alloys. 85

The herein described alloys may be cast, 90 rolled, extruded or otherwise shaped by methods commonly used for magnesium base alloys and the proportions of the alloying ingredients are to be governed by the particular application in view. Compositions which are suitable for extrusion may contain from 0.1 to 15 per cent of cadmium, from 0.1 to 15 per cent of zinc, and from 0.1 to 2.5 per cent of manganese. As a general purpose light weight alloy, suitable compositions are from 0.1 to 10 per cent of cadmium, zinc 0.5 to 10 per cent, and 0.1 to 2 per cent of manganese, 95 100

the balance being magnesium. It is preferable, however, to employ from 0.5 to 1.5 per cent of manganese and from 2 to 8 per cent of zinc and from 2 to 10 per cent of cadmium.

- 5 Another example of alloys within the scope of this invention which are easily press forged consist of from 2 to 6 per cent of cadmium, 2 to 4 per cent of zinc, and 1 per cent of manganese, the balance being magnesium. The new quaternary alloys consisting of from 2 to 10 per cent of cadmium, from 0.1 to 3 per cent of zinc, and from 0.5 to 1.5 per cent of manganese, the balance being magnesium, are easily hammer forged in heated 10 condition. For exceptionally high tensile strength the manganese content may be from 0.75 to 2 per cent, while that of cadmium may be from 6 to 10 per cent, and that of zinc from 2 to 10 per cent. For example, an 15 alloy consisting of magnesium, cadmium, zinc, and manganese wherein the quantity of magnesium in the alloy is 85 per cent, that of cadmium, zinc, and manganese is 10, 4, and 1 per cent, respectively, has a tensile 20 strength and yield point of 47,700 lbs./sq. in. and 35,000 lbs./sq. in., respectively, in the extruded condition.

These new alloys may be produced by melting the ingredients together under a suitable 30 flux, in a closed chamber or in an inert atmosphere, according to the usual methods of preparing magnesium alloys. The manganese may be also added to magnesium by allowing molten magnesium to react upon a 35 reducible manganese compound and subsequently the other alloying ingredients may be added.

Other modes of applying the principle of 40 my invention may be employed instead of the one explained, change being made as regards

the proportions of the ingredients employed within the limits specified, provided the ingredients stated by any of the following claims or the equivalent of such stated ingredients be employed.

I therefore particularly point out and distinctly claim as my invention:—

1. As a new product, a magnesium alloy composed of the metals magnesium, cadmium, zinc, and manganese wherein the magnesium content is in excess of 75 per cent, that of cadmium and zinc each is from 0.1 per cent to 15 per cent, and that of manganese from 0.1 to 2.5 per cent.

2. As a new product, a magnesium alloy 80 consisting of 0.1 to 10 per cent of cadmium, from 0.5 to 10 per cent of zinc, from 0.1 to 2 per cent of manganese, the balance being magnesium.

3. As a new product, a magnesium alloy 85 consisting of from 2 to 10 per cent of cadmium, from 2 to 8 per cent of zinc, and from 0.1 to 2.5 per cent of manganese, the balance being magnesium.

4. As a new product, a magnesium alloy 90 consisting of from 2 to 6 per cent of cadmium, from 2 to 4 per cent of zinc, and approximately 1 per cent of manganese, the balance being magnesium.

5. As a new product, a magnesium alloy 95 consisting of from 2 to 10 per cent of cadmium, from 0.1 to 3 per cent of zinc, and from 0.5 to 1.5 per cent of manganese, the balance being magnesium.

6. As a new product, a magnesium alloy 100 consisting of 6 to 10 per cent of cadmium, from 2 to 10 per cent of zinc, from 0.75 to 2 per cent of manganese, the balance being magnesium.

JOHN A. GANN. 105

45

110

50

115

55

120

60

125

65

130